

Patented May 22, 1934

1,960,177

# UNITED STATES PATENT OFFICE

1,960,177

## LAMINATING PROCESS

Josef Weber and Franz Hengstebeck, Essen, Germany, assignors, by mesne assignments, to Th. Goldschmidt Corporation, New York, N. Y., a corporation of Delaware

No Drawing. Original application June 2, 1931, Serial No. 541,734. Divided and this application March 17, 1932, Serial No. 599,586. In Germany February 2, 1929

1 Claim. (Cl. 144—309)

This invention relates to laminating processes; and it comprises a method of making improved laminated articles such as plywood, wherein a sheeted adhesive is assembled between layers of material, such as wood, heat and pressure are applied to the assemblage thereby softening and fusing said adhesive to form a mobile liquid and the said adhesive is then allowed to harden in situ to unite said layers with a hard insoluble bond; 5 the said sheeted adhesive comprising an open textured reinforcing paper sheet impregnated with a dried, potentially reactive condensation product of an aldehyde with a phenol fusible at temperatures not substantially exceeding 130° C. 10 to give a homogeneous, easy flowing liquid and said condensation product being formed in the presence of aqueous caustic alkali sufficient to maintain the products in solution during and after condensation; all as more fully hereinafter 15 set forth and as claimed.

In the usual method of cementing wood to wood, including affixing veneers and making plywood, the surfaces are treated with a solution of glue and setting performed under heat and pressure. Setting is really a removal of water and where extensive surfaces are united, the water is taken up by the wood. Most liquid glues contain large proportions of water and in making plywood, the amount of water to be dissipated in the glue used may be as high as 30 or 40 per cent of the weight of the wood to be joined. In building up plywood assemblages, the glue is applied to inner layers and the water is taken up by proximate layers thereby necessarily swelling these. At this stage in the operation the product includes a swollen inner wood layer connected to less moist outer layers or plies. In drying, the swollen inner layers tend to shrink to their original proportions thereby setting up heavy stresses and causing warping. Making plywood in this manner by the assemblage of successive laminae of wood with intermediate drying is a tedious operation and the product is apt to be irregular. The whole assemblage must be finally dried and unless this final drying, as well as the intermediate dryings, be conducted with exceptional care and skill an unsatisfactory product results. It may be warped, mottled or exhibit fissures (incipient cleavage). In order to obviate these difficulties it has been proposed to manufacture plywood and affix veneers by employing between the layers of wood a cementing layer in the form of glue-surfaced sheets of paper, of fabric, or even of wood. In making the cementing layer, suitable sheets 50 are passed through a glue solution and afterwards dried so as to form adhesive surfaced sheets adapted to be interposed between the wood plies. Using sheets of this character the amount of

water necessary can be limited to that required to make the surface of the sheets sticky; and this is 60 an advantage. This method while better than the more common procedure of cementing by liquid glue directly applied is nevertheless open to certain objections. For one thing in the final product, there is an intermediate structural element between the wood plies. For another, plywood made in this manner when subjected to changes in temperature and moisture conditions frequently tends to split apart along the plane of the intermediate fabric layer; the layer carrying 70 the glue on its surfaces. Unless the glue is waterproofed in some manner, the dried layer is not resistant to the action of moisture.

In affixing veneers and in making plywood it is desirable to have the wood layers as close together, 75 face to face, as possible, restricting the amount of intermediate adhesive to that sufficient to even out surface irregularities. And it is desirable to have an adhesive requiring in setting the dissipation of no great amount of water or of a volatile 80 solvent; of any amount causing substantial swelling in the wood. These results are accomplished in the present invention wherein is provided a thin substantially dry, substantially homogeneous lamina of adhesive usually containing a tenuous 85 fiber reinforcement in negligible amount; the adhesive being solid at the ordinary temperature, softening and fusing to a mobile liquid at higher temperatures and finally setting to a hard in-fusible, permanent form on exposure to temperatures such as are used in making plywood, say at 90 130° C.

For our purpose we use a particular condensation product of a phenol and formaldehyde in the presence of a rather large amount of alkali; this 95 alkali serving both as a catalyst in inducing condensation and having certain other functions. As the phenol, ordinary phenol may be used or one of the cresols. In lieu of formaldehyde, acetaldehyde or other aldehydes may be employed. However, ordinary phenol and ordinary formaldehyde, as the commercial 40 per cent solution, give good results. On dissolving equivalent amounts of phenol and formaldehyde (in solution) in 40 per cent caustic soda lye using 100 the amount of lye necessary for solution, a satisfactory preparation can be made for the present purposes. With a batch of 94 kilograms of phenol and 100 kilograms of commercial 30 per cent formaldehyde solution about 17 kilograms of 40 105 per cent NaOH solution give a good preparation. This liquid is kept warm for a time say at 80° C. for 1½ hours, with constant stirring until an easy flowing oily dark liquid is obtained. The viscosity depends upon the time of heating but is rather 110 low in any event. The exact viscosity desired can 115

be obtained by interrupting the heating and then 5 reaches a point somewhere around 130° C. when cooling. Because of the solvent influence of the excess of alkali and of the water present, no separation into two layers is produced. The oily liquid can be dried to a substantially dry material at temperatures below about 100° C. without going into the final insoluble resin. Ordinarily it is desired to dry the material to about 2 per cent water. By proper manipulation the dried material 10 may be made in thin sheets. These sheets at the ordinary temperature are not tacky but are somewhat hygroscopic in the sense that they will take up more water from the air. Ordinarily the amount taken up will give a final product of about 5 to 8 per cent; this varying with the 15 humidity. With this content of water the product is flexible and not sticky or tacky and the sheets can be packaged, shipped and stored as rolls without danger of adhesion.

20 As so far described, the sheets are made without the use of a reinforcement but for manufacturing reasons it is better to employ a tenuous reinforcement of fiber in negligible amount; an amount insufficient to produce a substantial intervening 25 layer between the sheets of wood ultimately to be united. As this reinforcement we employ an open textured, thin tissue paper, or like sheeted material. With the aid of this paper it is possible to produce the present material by ordinary 30 manufacturing operation in a continuous manner; a web of paper passing first through the initial condensation product, past equalizing rolls and then through drying apparatus. Drying is usually so conducted as to give about 2 per cent water in the dry material and sufficient exposure to air is then permitted to allow assumption of the full amount of "water of condition"; usually about 8 per cent. The proportion of fiber to adhesive varies but is usually in about the ratio 40 of 1:2. With thin open textured paper in this proportion the final sheeted product has a substantially continuous body of adhesive. In making such completely and uniformly impregnated sheets which are in fact continuous films of adhesive, the thickness and porosity or open texture of the reinforcing sheet are so correlated with the liquidity or viscosity of the oily liquid condensation product containing caustic soda as to insure a complete, continuous and uniform impregnation. 45 When this relation is properly established the oily liquid penetrates all the pores of the reinforcing medium and it is only necessary to apply the proper amount of liquid to give the desired ratio of condensation product to the reinforcing material.

50 The presence of the caustic soda, (for which caustic potash may be substituted), in the composition in about the amount indicated gives a preparation which at the ordinary temperature is not tacky; is not hygroscopic enough to become moist and sticky in ordinary air. It does however take up a little water of condition; enough to make it flexible and easily handled. The dry composition on warming to a few degrees above 55 the ordinary temperature becomes plastic enough to facilitate easy sheeting and on recooling is permanent; it can be stored, packaged and handled without trouble. In heating to fusion in use, probably the caustic soda and the small amount of water of condition present exercise a solvent action or contribute to fusion. The caustic soda solution produces condensation in making the initial oily liquid but it does not cause condensation much beyond this point with any reasonable degree of temperature until the heat

reaches a point somewhere around 130° C. when the catalytic action becomes extremely rapid. In the final product the caustic soda does not exist in any form making the article hygroscopic; nor is it necessary in making plywood to provide for the dissipation of the water present in the mixture. It is, in any event, small in amount being only about 5 to 8 per cent of the adhesive.

When the flexible sheeted adhesive (with or without reinforcement) is placed between two layers of wood in the usual way of affixing veneers or making plywood and heat and pressure are applied, the adhesive at first yields and softens, then fuses and is then taken up for the most part by the pores of the wood; finally solidifying in place. With about 8 per cent water in the material on fusing it forms a fairly mobile liquid readily taken up by pores as a whole; there being no segregation of solvent by the pores of the wood as there usually is with moist glue made plastic by heat. The alkali and water have a fluxing action but the melt is homogeneous. In the presence of the alkali and water, there is some reaction on the wood fiber contributing to the extremely perfect cohesive union ultimately secured.

95 On heating the assemblage of plies and adhesives up to, say, 130° C. the condensation products are converted into the final insoluble resin without much change in volume and with very little extrication of water; not enough to cause swelling or require any special care in subsequent drying.

100 Because of the properties of the present adhesive sheet it is possible to join a number of layers of plywood together simultaneously instead of successively as is the usual practice; thereby economizing time and labor.

105 While the invention has been particularly described in its use in cementing veneers and making plywood, the adhesive sheets of the present invention are advantageous in many other relations and may be used for general cementing purpose. Their use in forming a facing layer on various articles is advantageous.

110 This application is a continuation-in-part of our application, Serial No. 424,715, filed Jan. 30, 1930 and a division of our application, Serial No. 541,734, filed June 2, 1931.

115 What we claim is:

120 In the manufacture of plywood articles having at least two layers of wood united by an interposed hardened insoluble adhesive in interlocking engagement therewith, the process which 125 comprises warming a phenol and formaldehyde together in the presence of an aqueous caustic 130 soda solution under conditions suitable for producing a homogeneous, oily, liquid condensation product without the separation of an aqueous layer, impregnating a porous, open textured, thin tissue paper sheet with said product and drying 135 the impregnated paper; the amount of alkali present not being sufficient to give the dried sheet a tacky surface but being sufficient to cause absorption of from about 5 to 8 per cent of water of condition on exposure to air; assembling the resulting reinforced sheet of adhesive between layers of wood, applying pressure to said assemblage 140 while heating to a temperature not substantially exceeding 130° C. thereby softening and fusing said adhesive to form a mobile liquid and then hardening said adhesive in situ to unite said layers with a hard insoluble bond.

JOSEF WEBER.  
FRANZ HENGSTEBECK.

80

85

90

95

100

105

110

115

120

125

130

135

140

145

150